

Patented May 5, 1936

2,039,458

# UNITED STATES PATENT OFFICE

2,039,458

## ALUMINIUM ALLOYS

Josef Schulte, Bonn-on-the-Rhine, Germany, assignor to Vereinigte Leichtmetallwerke Gesellschaft mit beschränkter Haftung, Bonn-on-the-Rhine, Germany, a corporation of Germany

No Drawing. Application March 1, 1935, Serial No. 8,808. In Germany March 2, 1934

### 2 Claims. (Cl. 75—142)

This invention relates to aluminium alloys.

It is known that aluminium alloys with low contents of copper, magnesium and manganese attain very high mechanical strength values, especially when in the agehardened condition. These known alloys have a composition of about 3 to 5% of copper, 0.2 to 1% of magnesium and 0.2 to 1.5% of manganese. In order further to improve the mechanical properties of such alloys, the silicon content has been raised from the natural limits of impurity namely, 0.2 to 0.3% to up to 1.5%. It has also been proposed to increase the magnesium content of such alloys to about 1.2%.

Endeavours are however still being directed to improving still further the mechanical properties of these alloys, particularly for the purpose of saving weight in aircraft construction. In this connection, not only an increase in breaking strength, but also the raising of the elastic limit and yield point come into consideration. These properties can of course be improved to a certain extent by cold working, because the resulting consolidation also raises the yield point. Such procedure, however, can be applied to only a limited extent in practice, because elongation and capacity for undergoing deformation by mechanical treatment are naturally considerably lessened thereby. It is therefore a point of special importance, especially in the case of moving vehicles, to arrive at an improvement in the mechanical properties by suitably compounding the alloys.

It has now been ascertained, by comprehensive experiments, that particularly good results are furnished by alloys of the following composition—

|           | Percent      |
|-----------|--------------|
| Copper    | 3 to 5       |
| Magnesium | 1.3 to 1.4   |
| Silicon   | 0.4 to 0.7   |
| Manganese | 1.25 to 1.45 |
| Aluminium | Remainder    |

These alloys differ substantially from already known alloys by an accurately harmonized content of manganese, and also by a further increase in the magnesium content.

For example, an alloy containing:

|           | Percent   |
|-----------|-----------|
| Copper    | 4.0       |
| Magnesium | 1.35      |
| Silicon   | 0.65      |
| Manganese | 1.3       |
| Aluminium | Remainder |

after annealing at temperature of 510°, quenching and storing for 6 days, exhibits the following values:

|                  |                           |
|------------------|---------------------------|
| Yield point      | 33 to 36 kgs. per sq. mm. |
| Tensile strength | 48 to 54 kgs. per sq. mm. |
| Elongation       | 14 to 18%                 |

For comparison, it may be stated that a known alloy containing for example:

|           | Percent   |
|-----------|-----------|
| Copper    | 4.0       |
| Magnesium | 1.2       |
| Silicon   | 0.7       |
| Manganese | 1.2       |
| Aluminium | Remainder |

on being hardened in the same manner, exhibited a yield point of 31 to 33 kgs. per sq. mm., a tensile strength of 48 to 50 kgs. per sq. mm., and an elongation of 18 to 19%.

As is evident from the comparison of these data the yield point—a highly important technical property in aviation—is very notably increased by the new composition of the alloys. The very slight reduction in the elongation is of no moment, and is also counterbalanced by the not inconsiderable increase in tensile strength.

### I claim:

1. An aluminium alloy, which is age-hardenable by annealing, quenching and aging at room temperature, consisting of 3 to 5% of copper, 1.3 to 1.4% of magnesium, 0.4 to 0.7% of silicon and 1.25 to 1.45% of manganese, the remainder being aluminium.

2. An aluminium alloy as set forth in claim 1, consisting of 4% of copper, 1.35% of magnesium, 0.65% of silicon and 1.3% of manganese, the remainder being aluminium.

JOSEF SCHULTE.